

July 15, 1941.

J. A. WAINWRIGHT ET AL

2,249,069

PROCESS FOR PRODUCING LUSTER EFFECTS ON TEXTILES

Filed April 25, 1939

FIG. 3



FIG. 2



FIG. 1



J. A. WAINWRIGHT  
J. ALLAN

INVENTORS

*J. A. Wainwright & J. Allan*

ATTORNEYS

## UNITED STATES PATENT OFFICE

2,249,069

PROCESS FOR PRODUCING LUSTER  
EFFECTS ON TEXTILES

James Arthur Wainwright and John Allan,  
Spondon, near Derby, England, assignors to  
Celanese Corporation of America, a corpora-  
tion of Delaware

Application April 25, 1939, Serial No. 269,872  
In Great Britain May 9, 1938

10 Claims. (Cl. 8—63)

This invention relates to the treatment of textile materials, and more particularly to the production of ornamental effects on textile materials.

It has now been discovered that valuable ornamental effects may be obtained on textile fabrics or other textile materials by a process which comprises the operations, in either order, of locally applying to the textile material a substance which will precipitate albumen and applying to the textile material a composition containing albumen, a pigment and a dyestuff which has affinity for the textile material, and thereafter fixing the albumen on at least part of those portions of the textile material to which the precipitant for albumen was not applied. According to a modification of the invention valuable effects may be produced by applying to a textile material a composition containing albumen and a pigment but free from dyestuffs having affinity for the textile material, then locally applying to the textile material a substance which will precipitate albumen, and thereafter fixing the albumen on at least part of those portions of the textile material to which the precipitant for albumen was not applied. Particularly valuable results according to the invention may be obtained by applying both the precipitant composition and the pigment composition by printing, the design in which the pigment composition is applied being different from and in part overlapping that in which the precipitant composition is applied.

The precipitant for albumen acts as a resist so that the pigment is fixed on the textile material only on those portions of the textile material to which the precipitant for albumen is not applied. The fixation of the pigment is due to the fixation of the albumen, the albumen being converted to an insoluble envelope which surrounds the pigment particles and which is itself firmly fixed to the textile material. However, on those portions of the textile material to which the precipitant for albumen is applied, the albumen in the pigment composition is precipitated in a form which is non-adherent to the textile material and for this reason does not fix the pigment on the fibre. The unfixed pigment on these portions of the textile material may readily be removed by a scouring treatment.

Surprisingly, however, although the pigment is thus prevented from being fixed on the fibre by the application of the precipitant for albumen, dyestuff present in the pigment composi-

tion is not so prevented, even when the precipitant is applied before the pigment composition, with the result that the dyestuff colours the textile material over the whole of such portions 5 of the textile material to which it is applied, i. e., it colours both the portions to which the precipitant for albumen is applied and the portions to which the precipitant for albumen is not applied.

The resulting fabric therefore carries a pigmented design superimposed on the design in which the precipitant for albumen is applied, and, when a pigment composition containing a dyestuff is employed, is either coloured all over 15 its surface or carries a coloured design which is the design in which the pigment composition is applied.

Particularly valuable effects may be produced according to the process of this invention by 20 employing a white pigment and applying the process to lustrous fabrics, e. g., fabrics containing yarns of cellulose acetate or other organic derivatives of cellulose, since in this way 15 there may be obtained fabrics which carry a (pigmented) design of dull luster against a lustrous field, both the portions of dull luster and those of bright luster being coloured.

Suitable precipitants for albumen which may 30 be applied locally to the textile materials are citric acid, tartaric acid, zinc sulphate and ammonium nitrate. Such precipitants will, in general, be applied by printing thickened solutions thereof on the textile material. Suitable thickening agents are, for example, gum tragon, British 35 gum, locust bean thickening and water-soluble high viscosity hydroxyethyl ethers of cellulose as described in U. S. specification No. 195,-579 filed March 12, 1938. If desired, colouring 40 matters having affinity for the textile material may be incorporated in the precipitant composition. By this means, if the same colouring matter is employed in the pigment composition as in the precipitant composition, there may be obtained lighter shades in pigmented areas contrasting with deeper shades in the areas remaining free from pigment or, if different colouring 45 matters are employed in the two compositions, pigmented and non-pigmented areas which differ in colour may be produced.

As white pigments there may be employed 50 titanium dioxide, barium sulphate, lithopone and similar substances. Coloured pigments may be employed if desired in place of or in addition to white pigments. The dyestuff employed must,

as stated above, have affinity for the textile material treated. Dyestuffs having affinity for cellulose acetate materials may be of the aminoanthraquinone series, the azo series or the nitro diarylamine series. The dyestuffs in general which are marketed under the trade name "S. R. A." are especially suitable for the treatment of cellulose acetate materials.

The fixation of the albumen on the portions of the textile material to which the precipitant for albumen is not applied may be effected by heating the materials, preferably by a steaming operation at atmospheric or superatmospheric pressure. If the pigment composition is applied before the precipitant composition, the fabric must not be heated between the application of the two compositions. Where it is desired to obtain a design in dull luster on a lustrous cellulose acetate fabric, it is important that the fixing treatment should not dull the luster of those portions of such fabric to which the pigment is not fixed. A suitable steaming operation in these circumstances is one effected at atmospheric pressure.

As a modification of the process there may be employed in the pigment composition, instead of a dyestuff having affinity for the textile materials, a compound which though not itself a dyestuff is capable of being readily converted to a dyestuff on the materials. Thus the pigment composition may contain a component of an azo dyestuff, a leuco derivative of a vat dyestuff or an ester of a leuco derivative of a vat dyestuff, and the conversion to the final dyestuff on the materials effected as a subsequent operation.

While the invention has been described with particular reference to the treatment of cellulose acetate materials and materials having a basis of other organic derivatives of cellulose, it will be appreciated that it may also be applied to the treatment of other materials, e. g. regenerated cellulose materials, silk, cotton or wool.

The following examples illustrate the invention:

#### EXAMPLE 1 (a)

A cellulose acetate satin fabric is printed locally with a precipitant composition comprising 20 parts by weight of tartaric acid and 80 parts by weight of a 10% aqueous solution of gum tragacanth, and the fabric is dried. The fabric is then printed in a different design and so that parts of the two designs overlap, with the following pigment composition:

| Parts by weight                                                            |    |  |
|----------------------------------------------------------------------------|----|--|
| 10% aqueous paste of $\alpha$ -( $\beta$ -hydroxyethyl)-aminoanthraquinone | 1  |  |
| Aqueous dispersion of titanium dioxide containing 50% of titanium dioxide  | 30 |  |
| Aqueous albumen containing 50% of albumen                                  | 20 |  |
| 1% aqueous solution of gum tragacanth                                      | 49 |  |

The fabric is thereafter dried, steamed for 6 minutes at atmospheric pressure, washed to remove unfixed titanium dioxide, rinsed and dried. The finished fabric exhibits a design of delustered pink and lustrous pink. That is to say, where the pigment composition print is superimposed on the precipitant composition print a lustrous pink is obtained and the remainder of the fabric has the design of the pigment composition print as a delustered pink.

#### EXAMPLE 1 (b)

A cellulose acetate satin fabric is treated simi-

larly to that of Example 1 (a) except that 1 part by weight of a 10% aqueous paste of 1.5-dihydroxy-4-methylamino-8-aminoanthraquinone is employed in the place of the paste of  $\alpha$ -( $\beta$ -hydroxyethyl)-aminoanthraquinone. The finished fabric exhibits a design of delustered blue and lustrous blue.

#### EXAMPLE 2 (a)

A cellulose acetate satin fabric is printed locally with the following precipitant composition from a large-check object roller:

| Parts by weight                                                            |    |  |
|----------------------------------------------------------------------------|----|--|
| Tartaric acid                                                              | 20 |  |
| 7.5% aqueous solution of a water-soluble hydroxyethyl ether of cellulose   | 80 |  |
| 10% aqueous paste of $\alpha$ -( $\beta$ -hydroxyethyl)-aminoanthraquinone | 1  |  |

The fabric is then dried and printed with the following pigment composition from a small-check cover roller:

| Parts by weight                                                            |       |  |
|----------------------------------------------------------------------------|-------|--|
| 10% aqueous paste of $\alpha$ -( $\beta$ -hydroxyethyl)-aminoanthraquinone | 6.75  |  |
| Aqueous dispersion of titanium dioxide containing 50% titanium dioxide     | 20    |  |
| Aqueous albumen containing 50% of albumen                                  | 15    |  |
| 1% aqueous solution of gum tragacanth                                      | 58.25 |  |

The fabric is thereafter dried, steamed for 6 minutes at atmospheric pressure, washed to remove unfixed titanium dioxide, rinsed and dried. The finished fabric exhibits pink lustrous areas with small checks of lustrous red print where the cover roller has fallen on the areas printed with precipitant composition, together with pink delustered small checks on lustrous uncoloured areas where the cover roller has fallen on areas free from precipitant composition.

#### EXAMPLE 2 (b)

A cellulose acetate satin fabric is treated similarly to that of Example 2 (a) except that the following compositions are employed:

| Precipitant composition                                                  |    |  |
|--------------------------------------------------------------------------|----|--|
| Tartaric acid                                                            | 20 |  |
| 7.5% aqueous solution of a water-soluble hydroxyethyl ether of cellulose | 80 |  |
| 10% aqueous paste of 1.5-dihydroxy-4-methylamino-8-aminoanthraquinone    | 1  |  |

| Pigment composition                                                    |    |  |
|------------------------------------------------------------------------|----|--|
| 10% aqueous paste of 1.5 dihydroxy-4-methylamino-8-aminoanthraquinone  | 1  |  |
| Aqueous dispersion of titanium dioxide containing 50% titanium dioxide | 20 |  |
| Aqueous albumen containing 50% of albumen                              | 15 |  |
| 1% aqueous solution of gum tragacanth                                  | 64 |  |

The fabric exhibits a similar effect to that produced in Example 2 (a) except that light blue and dark blue shades are present in place of the pink and red respectively.

#### EXAMPLE 2 (c)

A cellulose acetate satin fabric is treated similarly to that of Example 2 (a) using the precipitant composition of that example and the pigment composition of Example 2 (b). The finished fabric exhibits small checks of lustrous purple print on pink lustrous areas where the

cover roller has fallen on the areas carrying precipitant composition, together with blue delustered small checks on lustrous uncoloured areas where the cover roller has fallen on areas free from precipitant composition.

EXAMPLE 2 (d)

A cellulose acetate satin fabric is treated similarly to that of Example 2 (a) using the following precipitant composition:

|                                                                          | Parts by weight |
|--------------------------------------------------------------------------|-----------------|
| Tartaric acid                                                            | 20              |
| 7.5% aqueous solution of a water-soluble hydroxyethyl ether of cellulose | 80              |
| 10% aqueous paste of 2.4-dinitro-4'-amino diphenylamine                  | 2               |

and the pigment composition of Example 2 (b). The finished fabric exhibits small checks of lustrous green print on yellow lustrous areas where the cover roller has fallen on areas carrying precipitant composition, together with blue delustered small checks on lustrous uncoloured areas where the cover roller has fallen on areas free from precipitant composition.

EXAMPLE 3

A cellulose acetate satin fabric is treated similarly to that of Example 2 (a) using the following precipitant composition:

|                                                                                         | Parts by weight |
|-----------------------------------------------------------------------------------------|-----------------|
| Tartaric acid                                                                           | 20              |
| 7.5% aqueous solution of a water-soluble high viscosity hydroxyethyl ether of cellulose | 80              |

and the following pigment composition:

|                                                                           | Parts by weight |
|---------------------------------------------------------------------------|-----------------|
| 10% aqueous paste of 2.4-dinitro-4'-amino diphenylamine                   | 2               |
| 10% aqueous paste of Monastral Blue                                       | 1               |
| Aqueous dispersion of titanium dioxide containing 50% of titanium dioxide | 30              |
| Aqueous albumen containing 50% of albumen                                 | 20              |
| 1% aqueous solution of gum tragacanth                                     | 40              |

The finished fabric exhibits small checks of lustrous yellow print on lustrous uncoloured areas where the cover roller has fallen on areas carrying precipitant composition, together with green delustered small checks on lustrous uncoloured areas where the cover roller has fallen on areas free from precipitant composition.

EXAMPLE 4

A cotton or regenerated cellulose fabric is printed locally with a composition containing 20 parts by weight of tartaric acid and 80 parts by weight of a 10% aqueous solution of locust bean thickening, and the fabric is dried. The fabric is then printed in a different design and so that parts of the two designs overlap, with the following pigment composition:

|                                                                        | Parts by weight |
|------------------------------------------------------------------------|-----------------|
| Diazo Fast Red 7BL                                                     | 1.5             |
| Aqueous dispersion of titanium dioxide containing 50% titanium dioxide | 30              |
| Aqueous albumen containing 50% of albumen                              | 20              |
| 10% aqueous solution of locust bean thickening                         | 48.5            |

The fabric is thereafter dried, steamed for 30

minutes at atmospheric pressure, washed to remove unfixed titanium dioxide, rinsed and dried. The fabric exhibits a design of delustered pink and lustrous pink.

- 5 In any of the above examples the order of applying the compositions may be reversed, it being understood that if the pigment composition is applied before the precipitant composition the fabric is neither dried nor steamed between the application of the two compositions. Example 5 specifically illustrates this method of carrying out the invention.

EXAMPLE 5

A cotton or regenerated cellulose fabric is printed with the following composition:

|                                        | Parts by weight |
|----------------------------------------|-----------------|
| Rapidogen Scarlet R                    | 4               |
| Glycine A                              | 3               |
| Indigosol Developer GA                 | 5               |
| Rapidogen Developer N                  | 12              |
| Titanium dioxide                       | 10              |
| Aqueous albumen containing 50% albumen | 15              |
| Starch gum tragacanth thickening       | 40              |
| Water                                  | 11              |

The fabric is then printed in a design covering part of the original print with a composition comprising 20 parts by weight of tartaric acid and 80 parts by weight of a 10% aqueous solution of locust bean thickening. The fabric is thereafter dried, steamed for 5-10 minutes at atmospheric pressure, washed to remove unfixed titanium dioxide, soaped, rinsed and dried. The fabric exhibits a design of delustered scarlet and lustrous scarlet.

In the appended claims the expression "a coloring agent for the textile material" is to be understood as meaning a dyestuff which has affinity for the textile material or a compound which is capable of being readily converted into such a dyestuff on the textile material.

The accompanying drawing illustrates the steps making up the process of the present invention. Figure 1 illustrates a method of producing a large printed design, on only the colored parts of which is superimposed a small contrasting design; it thus illustrates the methods of Examples 1a, 1b and 4. Figure 2 illustrates the production of designs by the methods of Examples 2a, 2b, 2c and 2d. Figure 3 illustrates the production of designs according to the method of Example 3.

Figure 1a represents fabric after the first step in which a precipitant composition is applied by printing as a small design over the whole of the fabric, areas 4 (diagonally ruled) being covered by the composition; Figure 1b represents the fabric after the step in which an albumen composition containing a dyestuff and a delustering pigment is applied in a large design to cover areas 5 (vertically ruled); and Figure 1c represents the finished fabric, after steaming and washing, where the large design of colored and delustered areas 6 (vertically ruled with continuous and with broken lines) stands out on a background of plain fabric and carries the small design of similarly colored non-delustered areas 7 (vertically ruled with continuous lines only).

Figure 2a represents fabric after the first step in which a precipitant composition containing a dyestuff is applied in a large design covering areas 8 (diagonally ruled from lower left to upper right); Figure 2b represents the fabric after the

step in which an albumen composition containing a dyestuff and a delustering pigment is applied in a small design over the whole of the fabric, covering areas 9 (diagonally ruled from upper left to lower right); and Figure 2c represents the fabric after steaming and washing where the large design consists of nondelustered areas 10 consisting of small design areas 11 (solid black) colored by the joint action of the dyestuff of both compositions, in a field 12 (diagonally ruled with continuous lines only) colored only by the dyestuff of the precipitant composition, and the background 13 consists of plain fabric carrying the small design as delustered areas 14 (diagonally ruled with continuous and with broken lines) colored only by the dyestuff of the albumen composition.

Figure 3a represents a fabric after the first step in which a precipitant composition is applied in a large design, covering areas 15 (diagonally ruled from lower left to upper right); Figure 3b represents the fabric after the step of applying an albumen composition containing a dyestuff, a colored pigment and a delustering pigment in a small design over the whole of the fabric, covering areas 16 (diagonally ruled from upper left to lower right); and Figure 3c represents the fabric after steaming and washing, where the large design consists of areas 17 consisting of non-delustered small design areas 18 (diagonally ruled with continuous lines only), colored only by the dyestuff, in a field of plain fabric, and the background 19 consists of plain fabric carrying delustered small design areas 20 (diagonally ruled with continuous and broken lines), colored by the joint action of the dyestuff and the colored pigment.

Having described our invention, what we desire to secure by Letters Patent is:

1. Process for the production of effects on textile fabrics or other textile materials, which comprises the operations, in either order, of locally applying to a textile material a substance which will precipitate albumen and applying to the textile material a composition containing albumen, a pigment and a coloring agent for the textile material the design in which the pigment composition is applied in part overlapping that in which the precipitant is applied, and thereafter fixing the albumen on at least part of those portions of the textile material to which the precipitant for albumen was not applied.

2. Process for the production of effects on textile fabrics or other textile materials, which comprises applying to a textile material a composition containing albumen and a pigment, then locally applying to the textile material a substance which will precipitate the albumen the design in which the pigment composition is applied in part overlapping that in which the precipitant is applied, and thereafter fixing the albumen on at least part of those portions of the textile material to which the precipitant for albumen was not applied.

3. Process for the production of effects on textile fabrics or other textile materials having a basis of a cellulose derivative, which comprises the operations, in either order, of locally applying to the textile material a substance which will precipitate albumen and applying to the textile material a composition containing albumen, a pigment and a coloring agent for the textile material the design in which the pigment composition is applied in part overlapping that in which the precipitant is applied, and thereafter fixing

the albumen on at least part of those portions of the textile material to which the precipitant for albumen was not applied.

4. Process for the production of effects on textile fabrics or other textile materials, which comprises the operations, in either order, of locally printing on a textile material a substance which will precipitate albumen and printing on the textile material a composition containing albumen, a pigment and a coloring agent for the textile material, the design in which the pigment composition is applied being different from and in part overlapping that in which the precipitant is applied, and thereafter heating the materials so as to fix the albumen on at least part of those portions of the textile material to which the precipitant for albumen was not applied.

5. Process for the production of effects on textile fabrics or other textile materials, which comprises the operations, in either order, of locally applying to a textile material a substance which will precipitate albumen and applying to the textile material a composition containing albumen, a pigment and a coloring agent for the textile material the design in which the pigment composition is applied in part overlapping that in which the precipitant is applied, and thereafter heating the materials under a pressure which is at least as great as atmospheric pressure so as to fix the albumen on at least part of those portions of the textile material to which the precipitant for albumen was not applied.

6. Process for the production of effects on textile fabrics or other textile materials, which comprises applying to a textile material a composition containing albumen and a pigment, then locally applying to the textile material a substance which will precipitate the albumen the design in which the pigment composition is applied in part overlapping that in which the precipitant is applied, and thereafter steaming the material under a pressure which is at least as great as atmospheric pressure so as to fix the albumen on at least part of those portions of the textile material to which the precipitant for albumen was not applied.

7. Process for the production of effects on textile fabrics or other textile materials, which comprises the operations, in either order, of locally applying tartaric acid to a textile material, and applying to the textile material a composition containing albumen, a pigment and a coloring agent for the textile material the design in which the pigment composition is applied in part overlapping that in which tartaric acid is applied, and thereafter fixing the albumen on at least part of those portions of the textile material to which the tartaric acid was not applied.

8. Process for the production of effects on textile fabrics or other textile materials, which comprises the operations, in either order, of locally printing on a textile material a thickened solution of a substance which will precipitate albumen and printing on the textile material a composition containing albumen, a pigment and a coloring agent for the textile material, the design in which the pigment composition is applied being different from and in part overlapping that in which the precipitant is applied, and thereafter fixing the albumen on at least part of those portions of the textile material to which the precipitant for albumen was not applied.

9. Process for the production of effects on textile fabrics or other textile materials, which comprises the operations, in either order, of locally

applying to a textile material a substance which will precipitate albumen and applying to the textile material a composition containing albumen, a white pigment, and a coloring agent for the textile material the design in which the pigment composition is applied in part overlapping that in which the precipitant is applied, and thereafter fixing the albumen on at least part of those portions of the textile material to which the precipitant for albumen was not applied.

10. Process for the production of effects on textile fabrics or other textile materials, which comprises the operations, in either order, of locally applying to a textile material a composi-

tion comprising both a substance which will precipitate albumen and a dyestuff having affinity for the textile material, and applying to the textile material a composition containing albumen, a pigment and a coloring agent for the textile material the design in which the pigment composition is applied in part overlapping that in which the precipitant is applied, and thereafter fixing the albumen on at least part of those portions of the textile material to which the precipitant for albumen was not applied.

JAMES ARTHUR WAINWRIGHT.  
JOHN ALLAN.

CERTIFICATE OF CORRECTION.

Patent No. 2,249,069.

July 15, 1941.

JAMES ARTHUR WAINWRIGHT, ET AL.

It is hereby certified that error appears in the printed specification of the above numbered patent requiring correction as follows: Page 3, first column, line 47, in the table, for

1% aqueous solution of gum tragon ----- 40"  
read --1% aqueous solution of gum tragon ----- 47--; and that the said Letters Patent should be read with this correction therein that the same may conform to the record of the case in the Patent Office.

Signed and sealed this 12th day of August, A. D. 1941.

(Seal)

Henry Van Arsdale,  
Acting Commissioner of Patents.